

## UNITED STATES PATENT OFFICE

2,298,127

## PROCESS OF PREPARING ARTIFICIAL FIBERS

Oskar Huppert, Chicago, Ill., assignor to The Glidden Company, Cleveland, Ohio, a corporation of Ohio

No Drawing. Original application May 13, 1940, Serial No. 334,920. Divided and this application March 10, 1941, Serial No. 382,577

3 Claims. (Cl. 18—54)

The present invention relates to the production of artificial fibers from soya protein, such as artificial wool and the like.

The present application is a division of application Serial No. 334,920, filed May 13, 1940.

In the manufacture of artificial protein fibers, a spinning solution of the protein is extruded through spinnerets into a coagulating bath and the fibers are then hardened. After hardening the fibers are washed, subjected to an after-treatment, and may be variously treated to produce the finished fiber.

In the case of casein, for example, the fibers, after hardening, do not stick together and may be subjected to washing and the after-treatment without any particular difficulty. In the case of soya protein fibers, however, the individual fibers or filaments after hardening are sticky and adherent with the result that they stick together to form a coherent mass, thereby preventing successful after-treatment, carding and the like.

It is, therefore, an object of the present invention to overcome the aforementioned sticking of the hardened soya protein fiber.

It is a further object of the present invention to treat the hardened films before washing or other treatments to overcome the aforementioned sticking.

The invention is applicable to any fiber prepared from soya protein. The fiber may be spun from suitable solutions of either hydrolyzed or unhydrolyzed protein. The spinning solution may also comprise in whole or in part a soya protein disulfide prepared in accordance with United States Patent No. 2,112,210. Such a protein disulfide is prepared by treating a soya protein hydrolysate with carbon disulfide at a hydroxyl ion concentration which corresponds at most to that of a solution of calcium hydroxide and then oxidizing the thus sulfurized protein to form the disulfide.

The objects of the present invention may be accomplished by subjecting the hardened fiber, before washing, to the action of nitrous acid. The action of the nitrous acid is such that the fibers lose their stickiness and may thereafter be washed, subjected to an after-treatment, and otherwise successfully handled. It is surprising that the strength, elasticity, and flexibility of the fibers are not diminished by the treatment with nitrous acid. On the contrary, they become more resistant to boiling water and take dyes more easily. By this treatment the fibers become hydrophobic permanently waterproof and fast to washing and dry cleaning.

The treatment with nitrous acid may be effected in any suitable way. The fibers may be immersed in a solution of nitrous acid for a short time. Preferably when the fibers are acid, such as when they are coagulated in an acid bath, they may be immersed in a solution of sodium nitrite or other suitable nitrous acid forming substance.

The following examples are illustrative.

## Example I

300 grams of hydrolyzed soya protein are dissolved in 1560 cc. of water with the acid of 15 grams of sodium hydroxide. This solution is allowed to ripen one or two days and the spinning 15 solution so obtained, after being freed of air, is spun into a coagulating bath of a combination of 25% sulfuric acid and 15% sodium sulfate. The fibers are then treated in a hardening bath containing 5% formaldehyde and 8% sodium chloride. The acid containing fibers, before washing 20 are then treated for 5 minutes in a 2% solution of sodium nitrite, after which they are washed. No sticking difficulty is encountered during the washing operation and the fibers may be subjected to an after-treatment and other operations 25 without encountering sticking difficulties.

## Example II

300 grams of hydrolyzed soya protein are added to 1410 cc. of water. 150 cc. of a 10% caustic soda solution is then added with agitation to dissolve the protein and to produce a pH of 9-10. The solution is warmed to 45° C. and at this temperature 35 23 cc. of carbon disulfide is added with vigorous stirring. The stirring is continued for half an hour, whereupon the pH drops to 6-7. Air is then bubbled into the solution at 60° C. with vigorous stirring for an hour. The solution is allowed to cool to room temperature while agitating. The spinning of the fibers, coagulation, hardening and nitrous acid treatment is therefore the same as in Example I.

It will be understood that the detailed procedures described are capable of variation and modification without departing from the spirit and scope of the invention defined in the appended claims.

I claim:

1. The process of preparing artificial fibers comprising spinning into a coagulating bath to form fibers a solution containing soya protein disulfide prepared by treating soya protein hydrolysate with carbon disulfide at a hydroxyl ion concentration which at most corresponds to that of a solution of calcium hydroxide and oxidizing the

thus sulfurized protein to produce the disulfide, hardening the fibers, subjecting the hardened fibers to the action of nitrous acid before washing, and then washing.

2. The process which comprises treating with nitrous acid a protein fiber containing a soybean protein disulfide resulting from the treatment of protein with carbon disulfide and oxidation of the

resulting sulfurized protein to form the disulfide.

3. The process which comprises treating with nitrous acid a disulfide protein fiber spun from a solution of a protein disulfide resulting from treatment of protein with carbon disulfide and oxidation of the resulting sulfurized protein to form the disulfide.

OSKAR HUPPERT.